

## UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS.

## HAIR FELT AND METHOD OF MAKING.

No Drawing.

Application filed September 12, 1923. Serial No. 662,220.

This invention has for its object to produce on a paper machine felt comprising a large proportion of hair of original length. This product when produced in accordance 5 with my invention is quite tough, but at the same time is somewhat open and porous in texture and may be saturated with asphalt, resins, gums, etc. of such nature and in such proportion as may be desired to give it characteristics suitable for roofing, flooring, shoe 10 stiffeners, or other products composed of saturated fibrous material.

The principal difficulty found in the use of large quantities of long hair such as that 15 comprising goat and cattle hair as it comes from tanneries is the strong tendency of the hair to become matted and lumpy in the machine so that uneven felt having weak spots therein is produced, and in attempts heretofore to produce a felt containing such hair, it has been necessary to set the beater roll 20 down so hard in beating out these lumps, that most of the hair has been cut or broken and consequently in the felt the hair was 25 relatively short. The more long hair that can be incorporated in the felt, however, the more porous the product and the stronger and tougher when saturated.

I have discovered that considerable quantities of hair may be successfully used to produce substantially uniform felt containing the hair in its original length, if in connection therewith some agent is used to individualize the hair while the furnish is 35 being prepared for felting. One such material which may be employed is short hair treated with caustic soda to form a slimy mass which coats the individual long hairs and permits them to slip on each other. As 40 an example of the way in which this may be used, the procedure may be as follows: twenty parts by weight of rags or other cellulosic material, thirty parts of goat or cattle hair as it comes from the tannery, and 45 six parts of caustic soda are placed in a beating engine with sufficient water to permit circulation, and are beaten with the beater roll down hard until the hair is quite short and the mixture forms a slimy mass. Fifty parts of long goat or cattle hair are 50 then added and the mixture beaten out to form a homogeneous mass with the beater roll raised just sufficiently so that the hair last added is kept long but is combed out

and coated with the other material. If the 55 individualizing agent is not used it is impossible to maintain the major portion of the long hair in its original length and yet separate it sufficiently to felt properly on the paper machine. By the use of this individualizing agent, however, and by careful adjustment of the beater roll, the hair may be combed out and coated with the individualizing material while maintained in its original length. Eight parts of alum may 60 then be added to the mixture which causes the slimy gelatinous mixture of short hair and hair wholly and partially dissolved in the caustic solution to be precipitated on the long hair. The stock may then be run into 65 the vat of the paper machine and sheeted in the usual manner.

The presence of the short hair and also the precipitated matter causes the felt to be somewhat more dense than would be the case 70 if they were not present and it also adds materially to the ease with which the stock is handled in the paper machine since they act to prevent the individualized fibers from matting together or becoming displaced 75 after having once been felted in the paper machine, pressure exerted thereon by the various pressure rolls being then ineffective to cause displacement of the fibers. This precipitated matter also acts to impart body 80 to the felt much increasing its strength when in dry condition. Practically all the individualizing agent so precipitated is aluminum gelatinous hydrate. The short hair alone also has some individualizing properties even though it is not completely dissolved by the caustic and the individualizing agent is thus composed of a mixture of 85 short hair and gelatinous slimy material.

In place of the rags, a mixture of rag and 90 sulphite pulp, or sulphate pulp alone may be employed and if it be desired to impart a more open texture to the material this may be effected by adding up to ten parts of wood flour or fine sawdust, preferably before the addition of that portion of the hair which is to be kept long in the final product. This wood flour or sawdust causes the stock to be freer and makes the saturating 95 of the product somewhat easier. The quantity of sulphate pulp or other cellulosic material, may be reduced if desired to as little as 10% and when this is done 20% of hair 100

which is beaten up short with the caustic to form an individualizing agent may be employed together with 70% of long hair. A small amount of cellulosic fiber such as 5 rags, chemical wood pulp, or screenings appears necessary in order that the stock may be caused to run successfully on the paper machine.

The action of the caustic on the short hair 10 is evidently partially to saponify the oil of the short hair fibers and partially to dissolve the hair, and to form a slimy mass which surrounds and coats the long hairs and causes them to slip by each other and become 15 thoroughly individualized and evenly distributed throughout the stock in the beater.

Hair as it comes from the tanneries is 20 usually matted and lumpy. During the process of de-hairing hides in the tanneries lime is usually used and the hair as it comes 25 from the de-hairing operation is wet and mixed with lime. As this mixture does not keep, it is the usual practice to wash out the lime and then dry the hair. Some lime may, 30 however, be left in the hair in its dry state. The presence of such lime, when carrying out the process of this invention does no harm, but indeed is often of distinct value since a cheaper grade of caustic may be used, 35 the cheaper grades of caustic usually containing a considerable portion of sodium carbonate which is causticized by the lime into caustic soda. During this action the lime itself is converted for the most part 40 into insoluble salts which are retained by the gelatinous matter precipitated by the alum, and act as a filler for the final product. Unwashed hair may thus be used successfully 45 in the process of this invention with the cheaper grades of caustic when it can be procured sufficiently promptly from the tannery to avoid spoiling, but washed hair may be employed with substantially the same results if lime be added to the beater.

45 Where the unwashed hair can be obtained, however, it should be somewhat cheaper than the washed hair.

Having thus described this invention it should be evident to those skilled in the art 50 that various changes and modifications might be made therein without departing from its spirit or scope as defined by the appended claims.

I claim:

55 1. Felt having the characteristics of wet paper machine fabrication, said felt com-

prising hair of original length, short hair, and cellulosic material.

2. A method which comprises beating out 60 hard a mixture of cellulosic material, hair, and caustic until the hair is short or partially dissolved to a slimy state, then adding long hair, beating out the long hair while retaining its original length until it is individualized by the mixture, and then felting 65 the stock on a paper machine.

3. The method which comprises individualizing long hair with a mixture containing 70 short and partially dissolved hair, and then felting the stock on a paper machine.

4. The method which comprises individualizing long hair with a mixture containing short and partially dissolved hair reduced 75 to a slimy state, and then felting the stock on a paper machine.

5. The method which comprises mixing long hair and an individualizing agent comprising short hair, and felting the stock on a paper machine.

6. The method which comprises mixing 80 long hair and a gelatinous individualizing agent comprising partially dissolved hair, and felting the stock on a paper machine.

7. The method which comprises mixing 85 long hair with an individualizing agent comprising short hair and caustic, and felting the stock on a paper machine.

8. The method which comprises mixing long hair with cellulosic material and an 90 individualizing agent comprising short hair and caustic, and felting the stock on a paper machine.

9. The method which comprises mixing long hair with an individualizing agent comprising partially dissolved hair forming a 95 gelatinous mixture, and felting the stock on a paper machine.

10. The method which comprises mixing long hair with an individualizing agent comprising short hair and caustic, precipitating 100 the individualizing agent on the hair, and felting the stock on a paper machine.

11. The method which comprises mixing long hair with cellulosic material and an individualizing agent comprising short hair 105 and caustic, precipitating the individualizing agent on the cellulosic material and long hair, and felting the stock on a paper machine.

In testimony whereof I have affixed my 110 signature.

ALBERT L. CLAPP.